

June 12, 1923.

1,458,290

H. C. HALL

## METHOD OF PREPARING METALLIC ALLOYS AND OF REFINING METALS AND ALLOYS

Filed Feb. 18, 1921



*Inventor:*

Horace Campbell Hall.

Attorney: AGH/Adam

Patented June 12, 1923.

1,458,290

# UNITED STATES PATENT OFFICE.

HORACE CAMPBELL HALL, OF DERBY, ENGLAND, ASSIGNOR TO ROLLS-ROYCE LIMITED, OF DERBY, ENGLAND, A BRITISH COMPANY.

## METHOD OF PREPARING METALLIC ALLOYS AND OF REFINING METALS AND ALLOYS.

Application filed February 18, 1921. Serial No. 446,114.

*To all whom it may concern:*

Be it known that I, HORACE CAMPBELL HALL, of Derby, England, have invented a certain new and useful Improved Method of Preparing Metallic Alloys and of Refining Metals and Alloys, of which the following is a specification.

This invention comprises an improved method of making metal alloys and of refining metals and alloys, more particularly useful where it is desired to add to a molten bath of the main constituent one or more ingredients of other metals (hereinafter referred to as the additive metals) which, although some of them may be of less specific gravity, are together of greater specific gravity than that of the main constituent. It is the common practice to cast the additive metals in convenient sized lumps and to throw such castings into the molten bath of the main constituent. When this method is adopted there is a tendency for some oxidation of such of the additive metals as are of less specific gravity than the main constituent to take place at the surface of the bath, due to such metals floating thereon and for the additive metals not to be evenly diffused throughout the main constituent.

According to this invention the additive metals are introduced into the molten bath of the main constituent in a granulated and oil-coated condition.

As an example in making an alloy of aluminium, zinc and magnesium there may be melted together 60 parts of aluminium and 30 parts of zinc whereupon there is dissolved therein 10 parts of magnesium, the resultant alloy being then granulated and introduced as additive to a bath of aluminium or other metal.

To bring the additive metals to the granulated and oil-coated condition required, they are melted together under charcoal or suitable flux or both in a manner well known, and then poured into a vessel containing oil. The vessel and oil are preferably of such size and quantity respectively in relation to the quantity of additive metals that the metal is cooled by the time it has fallen to the bottom of the vessel. To this end there may be arranged within the vessel containing the oil a horizontally placed metal roller rotating on its axis, the lower part of which is in the oil, the molten metal being caused to fall on to this roller which is fur-

nished, if necessary, with a scraper to prevent any metal adhering to its rising surface. A series of such rollers may be arranged so that the metal will fall or flow from one onto another. By means of rollers as above described the metal can be spread out in its descent, and caused to be more evenly dispersed throughout the oil.

The accompanying drawing shows a form of apparatus for effecting the granulation. <sup>65</sup> *a* is a tank containing oil, *b* is a steel roller actuated by the handle *b*<sup>1</sup>. *c* is a pot from which the metal is poured, *d* is a tray to receive granulated metal having vertical end members *d*<sup>1</sup> and handles *d*<sup>2</sup> to enable the tray <sup>70</sup> with the metal to be lifted from the tank. *e* is a scraper attached to one of the end members *d*<sup>1</sup> scraping any adhering metal from the surface of the roller emerging from the oil. *e*<sup>1</sup> is an overflow for oil from the <sup>75</sup> tank *a*.

The additive metals are by the means above described brought into a granulated condition with the granules coated with oil, the mass being frequently in a spongy condition. <sup>80</sup>

Moreover, due to its sudden cooling a certain amount of heat energy is entrapped in the metal, leaving it in a strained condition analogous to that obtaining in the case of <sup>85</sup> "Rupert's drops" these being formed, as is well known, by dropping molten glass into water. A less amount of heat energy is required to return the metal to its melting point. <sup>90</sup>

The effect of the above treatment is that when the additive metals are introduced into the bath of the main constituent a general and even diffusion of them, or a better diffusion than by methods hitherto in vogue, <sup>95</sup> is attained; and further the tendency to oxidation at the surface above referred to is eliminated or diminished.

This invention is useful not only for the purpose of altering the nature and qualities <sup>100</sup> of the main constituent, for example to harden or give greater strength to the final alloy, but also, when the addition of the additive metals is made, for the purpose of cleansing, refining by removing oxygen or <sup>105</sup> other impurities, or for the purpose of killing.

It is preferred to use for the purpose of this invention a pure mineral oil with a high flash point say not lower than 200° centi- <sup>110</sup>

grade, or not lower than 250° centigrade in the case where the additive metals are such as are usually selected for cleansing which generally cannot be melted under 700° centigrade.

What I claim as my invention and desire to secure as Letters Patent of the United States is:—

1. A method of preparing metal alloys and of refining metals and alloys consisting in introducing into a main molten constituent an additive metal or metals in a granulated and oil coated condition.

2. A method of preparing metal alloys and of refining metals and alloys consisting in melting an additive metal or metals, pouring same into an oil and introducing the

metal thus treated into a molten main constituent.

3. A method of preparing metal alloys and of refining metals and alloys consisting in melting an additive metal or metals, pouring same on to a revoluble member immersed in oil and introducing the additive metal or metals thus treated into a molten main constituent.

In witness whereof I have signed this specification in the presence of two witnesses.

HORACE CAMPBELL HALL.

Witnesses:

NORMAN HAY WALKER,  
VIOLET MAUD MASTERS.